

# UNITED STATES PATENT OFFICE.

CARL BACHE-WIIG, OF PORTLAND, MAINE.

## METHOD OF PREPARING PULP.

1,327,221.

Specification of Letters Patent. Patented Jan. 6, 1920.

No Drawing.

Application filed February 20, 1919. Serial No. 278,257.

To all whom it may concern:

Be it known that I, CARL BACHE-WIIG, a citizen of the United States, a resident of Portland, county of Cumberland, and State 5 of Maine, have invented an Improvement in Methods of Preparing Pulp, of which the following is a specification.

This invention relates to the production of pulp from cellulosic materials, including 10 pine wood, white pine, Norway pine, and other woods which are rich in resinous substances, including turpentine, all of which substances are herein expressly intended to be included in the general term, ligneous 15 matter.

In my application #231,204, filed April 27th, 1918, a method of preparing pulp is described whereby the ligneous matter for the most part is retained in order that its 20 weight may be added to the mass, and paper suitable for newsprint may be produced.

The method involves two treatments, which are carried on successively.

By the first treatment the cellulosic material composing the pulp is softened, that is to say, the ligneous matter is softened but not destroyed and the fibers are swollen and caused to separate.

By the second treatment the treated mass 30 is cooked with a bisulfite pulp forming liquor for a relatively short period of time, the process being checked before the destruction of the ligneous matter occurs.

A solution of sodium chlorid, NaCl, is employed, in the first treatment, and I find that this substance does not discolor the fiber but tends to whiten it, and when the treated mass is cooked with the bisulfite pulp forming liquor the fiber is not discolored and an 40 unbleached pulp is produced which is suitable for newsprint paper but which may be bleached if desired for the finer grades of paper.

The present invention is an improvement 45 on the aforesaid method and has for its object the production of unbleached pulp by a novel method involving the employment of a bisulfite pulp forming liquor or in other words the sulfite process, wherein the ligneous matter is removed from the fiber or substantially so, as contrasted to being saved and used as a constituent of the pulp.

By my present method a high grade of unbleached pulp may be made of high grade 55 cellulosic materials and a good unbleached pulp made of the low grades of cellulosic materials, such as the pines above noted,

which is suitable for newsprint paper, which can not be made by the method of my said application.

My present invention involves two treatments which I have carried on successively, similar to the method of the aforesaid application, although the object sought to be attained is the destruction and removal of the 60 ligneous matter.

The two successive treatments are or may be carried on at their maximum temperatures and for long periods of time, and particularly the first treatment where the period of time is continued for a great many 65 hours and until the ultimate result has been obtained.

In carrying out my first treatment, I may proceed as follows:

The material or substance employed, in small pieces or chips, is placed in a tank or digester, which may be opened or closed, and a softening agent, as a solution of sodium chlorid NaCl, is added, as for instance, 70 I may add water containing from one-half of one to 4 per cent. of sodium chlorid, and then heat the mass to a temperature from 70 C. to 110 C. for from 12 to 72 hours, the 75 temperature and the time being more or less variable depending upon the material used and the strength thereof, yet it will be understood that ordinarily the higher the temperature the shorter the time required and vice versa.

During this first treatment the ligneous matter is variously affected and in different degrees, as for instance the dissolution of some of the lignenes is hastened and of others is retarded; the vaporization of some 80 of the lignenes is also hastened and of others is retarded; the softening of some of the lignenes is hastened and of others is retarded; and probably all are more or less prepared for reaction with the bisulfite pulp 85 forming liquor which is employed in the subsequent treatment.

The cellulosic pieces or chips are saturated with the softening solution which is further utilized in the performance of the second 90 treatment of the method.

This solution is then drawn off or removed.

The same solution may be used repeatedly as a softening agent for a large number of 110 times, if desired.

As an example of the first treatment in case of the pines above noted, some of the resinous substances are dissolved in the so-

lution and others softened, and those of a volatile character, such as turpentine are vaporized and may be collected, if desired, and all which remain are more or less affected, 5 so that they are better prepared for reaction during the second treatment.

*The second treatment.*—The mass having been thus treated is then cooked with a bisulfite pulp forming agent, or a sodium chlorid solution depending upon that kind of paper the pulp is to be used, for instance, if during the first treatment a sodium chlorid solution is employed then during the second treatment a bisulfite liquor will be 10 employed and an unbleached pulp suitable for newsprint paper will be produced, or may be bleached for the finer grades of paper.

The strength of the bisulfite solution may 20 be such together with the time and temperature of cooking that the ligneous matter may practically be removed from the fiber.

The second treatment may continue for a period of time, say from 10 to 24 hours at a 25 temperature of from 110 degrees C. to 135 degrees C., but the longer the period of time and the lower the temperature within reasonable limits the better the pulp.

A reaction takes place between the sodium 30 chlorid with which the mass is saturated and the bisulfite liquor employed during the second treatment to which I attribute at least in part some of the advantages gained by this process.

35 I claim:—

1. The method of preparing pulp from 40 cellulosic material which consists in treating the material with sodium chlorid and subsequently cooking the mass with a bisulfite pulp forming liquor until substantially all the ligneous matter has been freed from the fiber.

2. The method of preparing pulp from 45 cellulosic material which consists in two successive treatments, first, treating the material with a sodium chlorid solution, and second in cooking the treated mass with a bisulfite pulp forming liquor until substantially all ligneous matter has been freed 50 from the fiber.

3. The method of preparing pulp from 55 cellulosic material in the form of chips, which consists in adding a solution of sodium chlorid to the material, heating the mass for a period of time to dissolve some of the ligneous matter in the solution, and vaporize some and prepare the remainder for subsequent reaction, then drawing off the solution and then cooking the treated mass 60 with a bisulfite pulp forming liquor until substantially all of the ligneous matter is freed from the fiber.

4. The method of preparing pulp from 65 cellulosic material in the form of chips, which consists in adding a solution of so-

dium chlorid to the material, heating the mass for a period of time to soften the ligneous matter, and dissolve some in the solution and prepare some for subsequent reaction, then drawing off the solution and then 70 cooking the treated mass with a bisulfite pulp forming liquor until substantially all of the ligneous matter is freed from the fiber.

5. The method of preparing pulp from 75 cellulosic material in the form of chips, which consists in adding a solution of sodium chlorid to the material, heating the mass for a period of time to soften the ligneous matter and dissolve some in the solution and vaporize some, and prepare some for subsequent reaction, then drawing off the solution, and then cooking the treated mass 80 with a bisulfite pulp forming liquor until substantially all of the ligneous matter is freed from the fiber.

6. The method of preparing pulp from 85 cellulosic material in the form of chips, which consists in adding a solution of sodium chlorid to the material, heating the 90 mass for a period of time to soften the ligneous matter and dissolve some in the solution, and prepare some for subsequent reaction, then drawing off the solution, and then cooking the treated mass with a bisulfite pulp forming liquor until 95 substantially all of the ligneous matter is freed from the fiber.

7. The method of preparing pulp from 100 cellulosic material in the form of chips, which consists in adding a solution of sodium chlorid to the material, heating the mass for a period of time to soften the ligneous matter and dissolve some in the solution, and prepare some for subsequent reaction, then drawing off the solution, and then cooking the treated mass with bisulfite pulp forming liquor until some of the ligneous matter has been dissolved by the liquor and substantially all is freed from 105 the fiber.

8. The method of preparing pulp from 110 cellulosic material, which consists in treating the material in the form of chips with 115 a water solution of sodium chlorid for a period of time and at a temperature, substantially as specified, and subsequently cooking the mass with a bisulfite pulp forming liquor for a period of time and at a temperature, substantially as specified, whereby substantially all ligneous matter is freed 120 from the fiber.

In testimony whereof, I have signed my name to this specification, in the presence of 125 two subscribing witnesses.

CARL BACHE-WIIG.

Witnesses:

CHARLES M. DRUMMOND,  
WADLEIGH B. DRUMMOND.